

1

3,515,652

### BRIGHT NICKEL PLATING

Malcolm J. Law, Greenford, England, assignor to John Preston and Company (Chemicals) Limited, Greenford, England  
No Drawing. Filed Nov. 25, 1966, Ser. No. 596,750  
Int. Cl. C23b 5/08, 5/46  
U.S. Cl. 204—49

13 Claims

### ABSTRACT OF THE DISCLOSURE

Bright nickel deposits are produced by electroplating nickel from an aqueous acidic solution of at least one nickel salt, the reaction product of an acetylene alcohol and an alkali metal perborate, and a water-soluble sulphy oxygen compound.

This invention relates to bright nickel plating. The invention is based on the discovery that on reacting in water acetylene alcohols with sodium perborate or any other alkali metal perborate capable of forming a borate derivative and incorporating this material in a nickel plating bath in combination with sulphy oxygen compounds of the sulphonic acid type, it is found to be very effective for promoting the formation of bright ductile nickel electro-deposits.

According to the invention there is provided a process for producing bright nickel deposits which comprises, electro-depositing nickel from an aqueous acidic solution of at least one nickel salt in which there is dissolved from 0.01 to 1.5 g./l. of a preformed borate compound consisting of the reaction product of an acetylene alcohol and an alkali metal perborate together with a water-soluble sulphy oxygen compound at a concentration of from 0.5 to 90 g./l.

By "preformed" we mean that the borate compound is produced before adding it to the plating solution.

The acetylenic alcohol may have the general formula



where  $M_1$  is a hydroxyl, hydroxymethyl or hydroxyethyl radical,  $M_2$  is a hydrogen or methyl radical and  $M_3$  is a methyl, hydroxymethyl, hydroxymethyl, methoxymethyl, diethylaminomethyl, morpholinomethyl or hydroxypropyne radical.

This alcohol may also be reacted with the perborate under reflux.

A typical method of reacting acetylenic alcohols with sodium perborate is as follows:

Equal molecular quantities of acetylenic alcohol and sodium perborate are taken. The acetylenic alcohol is made into a 50% solution form in water, placed in a reaction flask and heated to 85–95° C. under a reflux condenser.

The sodium perborate is added gradually until addition of total quantity of perborate has been made, reaction is then continued until gassing ceases and reaction product then gradually changes from a pale straw colour to a deep intense brown colour.

Whilst any of the water soluble acetylenic alcohols mentioned hereinafter in Table I can be used with success for producing a borate derivative, we have had particular success with 2-butyne-1:4-diol, 3-pentyne-1-ol, 2-methyl-3-butyne-2-ol, 1-pentyne-3-ol, 2-pentyne-1:4-diol.

Any of this particular group of chemicals is particularly effected when reacted with sodium perborate, especially 2-butyne-1:4-diol at a concentration of 0.01–0.5 gm.

2

of the borate derivative in combination with 0.5 to 30 g./l. of a sulphy oxygen compound per litre of the nickel solution.

Additions of the brighteners according to this invention have been used in the normal standard Watts type nickel electroplating bath. However, it was also found that they are equally effective in all other acid nickel electroplating baths and, therefore, the invention is applicable to any nickel electro-deposition operation that takes place from an aqueous acidic solution of one or more nickel salts.

Examples of acetylenic alcohols that we have successfully reacted with sodium perborate are given in Table I.

TABLE I

|    |                                                                                      |
|----|--------------------------------------------------------------------------------------|
| 15 | 2-propyne-1-ol $HC \equiv CCH_2CH$                                                   |
|    | 3-butyne-1-ol $HC \equiv CCH_2CH_2OH$                                                |
|    | 2-methyl-3-butyne-2-ol                                                               |
|    | 1-pentyne-3-ol $HC \equiv CCH(OH)CH_2CH_3$                                           |
|    | 3-methyl-1-pentyne-3-ol $HC \equiv C-C(CH_3)(OH)CH_2CH_3$                            |
| 20 | 3,5-dimethyl-1-hexyne-3-ol<br>$HC \equiv C-C(CH_3)(OH)CH_2(CH_3)_2$                  |
|    | 3-ethyl-1-heptyne-3-ol<br>$HC \equiv C-C(C_2H_5)(OH)CH_2CH_2CH_2CH_3$                |
|    | 1-ethynylcyclohexanol $HC \equiv C-C(OH)C_6H_{10}$                                   |
| 25 | 2-butyne-1:4-diol $HC \cdot CH_2C \equiv CCH_2OH$                                    |
|    | 4-methoxy-2-butyne-1-ol $HO \cdot CH_2C \equiv C \cdot CH_2OCH_3$                    |
|    | 1,4-dimethoxy-2-butyne $CH_3OCH_2C \equiv C \cdot CH_2OCH_3$                         |
|    | 3-hexyne-2-5-diol $CH_3CH(OH)C \equiv C \cdot CH(OH)CH_3$                            |
|    | 4-octyne-3,6-diol                                                                    |
| 30 | $CH_3CH_2OH(OH)C \equiv CCH(OH)CH_2CH_3$                                             |
|    | 2,5-dimethyl-3-hexyn-2,5-diol<br>$(CH_3)_2C(OH)C \equiv C-C(OH)(CH_3)_2$             |
|    | 3,6-dimethyl-4-octyne-3,6-diol<br>$CH_3CH_2C(CH_3)(OH)C \equiv CC(CH_3)(OH)CH_2CH_3$ |
| 35 | 4-diethylamino-2-butyne-1-ol<br>$HOCH_2C \equiv C \cdot CH_2N(C_2H_5)_2$             |
|    | 4-(N-morpholinyl)-butyne-1-ol<br>$HOCH_2C \equiv CCH_2N(C_2H_4)_2O$                  |
| 40 | 3-pentyne-1-ol $CH_3 \equiv CCH_2CH_2CH$                                             |
|    | 2,4-hexadyne-1-6-diol $HOCH_2C \equiv C-C \equiv CCH_2OH$                            |
|    | Acetylene dicarboxylic acid $HOOCC \equiv CCOOH$                                     |
|    | 2-pentyne-1:4-diol $HO \cdot CH_2-C \equiv C-CHOH-CH_3$                              |

As an example of borate compound, 450 g. of 2-butyne-1:4-diol dissolved in water and an equimolecular proportion of sodium perborate were heated to complete reaction. This reaction product can also be used for the production of a semi-bright nickel deposit from a Watts-type nickel solution in conjunction with an acetate.

50 The compounds listed in Table II are examples of the sulphy oxygen compounds which are used in conjunction with the reacted product of the acetylenic alcohols.

TABLE II

|    |                                                                                                          |
|----|----------------------------------------------------------------------------------------------------------|
| 55 | (1) Mononuclear aromatic sulphonnic acids and alkali metal ammonium, magnesium and nickel salts thereof. |
|    | Benzene monosulphonate $C_6H_5SO_3H$                                                                     |
|    | Sodium benzene monosulphonate $C_6H_5SO_3Na$                                                             |
|    | Nickel benzene monosulphonate $(C_6H_5SO_3)_2Ni$                                                         |
| 60 | Sodium para-toluene monosulphonate $CH_3C_6H_4SO_3Na$                                                    |
|    | Para-chlorobenzene sulphonate $ClC_6H_4SO_3H$                                                            |
|    | Sodium para-bromobenzene sulphonate $BrC_6H_4SO_3Na$                                                     |
|    | 1:2, dichlorobenzene sulphonate $Cl_2C_6H_3SO_3H$                                                        |
|    | 1:2, or 2.5 dichlorobenzene sulphonate sodium salt<br>$Cl_2C_6H_3SO_3Na$                                 |
| 65 | Meta-benzene disulphonate $C_6H_4(SO_3H)_2$                                                              |
|    | Sodium meta benzene disulphonate $C_6H_4(SO_3Na)_2$                                                      |
|    | Ortho-sulphobenzoic acid monoammonium salt<br>$HOCOC_6H_4SO_3NH_4$                                       |
| 70 | 1-amino-2,5-benzene disulphonate<br>$H_2NC_6H_3(SO_3H)_2$                                                |

Ortho-aminobenzene sulphonate  $\text{H}_2\text{NC}_6\text{H}_4\text{SO}_3\text{H}$   
 (2) Mononuclear aromatic sulphonics, and alkali metal, ammonium, magnesium and nickel salts thereof.  
 Sodium benzene sulphonate  $\text{C}_6\text{H}_5\text{SO}_2\text{Na}$   
 Sodium para-toluene sulphonate  $\text{CH}_3\text{C}_6\text{H}_4\text{SO}_2\text{Na}$

(3) Mononuclear aromatic sulphonamides and imides.  
 Benzene sulphonamide  $\text{C}_6\text{H}_5\text{SO}_2\text{NH}_2$   
 Para-toluene sulphonamide  $\text{CH}_3\text{C}_6\text{H}_4\text{SO}_2\text{NH}_2$   
 Ortho-benzoic sulphonamide  $\text{C}_6\text{H}_4\text{CONHSO}_2$   
 Benzyl sulphonamide  $\text{C}_6\text{H}_5\text{CH}_2\text{SO}_2\text{NH}_2$   
 Benzene sulphydroxamic acid  $\text{C}_6\text{H}_5\text{SO}_2\text{NHOH}$   
 N.N. dimethyl para-toluene sulphonamide  
 $\text{CH}_3\text{C}_6\text{H}_4\text{SO}_2\text{N}(\text{CH}_3)_2$   
 N.N. dicarboxyethyl benzene sulphonamide  
 $\text{C}_6\text{H}_5\text{SO}_2\text{N}(\text{C}_2\text{H}_4\text{CCO}_2)_2$

(4) Binuclear aromatic sulphonics and alkali metal, ammonium, magnesium and nickel salts thereof.  
 2-naphthalene monosulphonate  $\text{C}_{10}\text{H}_7\text{SO}_3\text{H}$

Thiophene sulphonate  $\text{C}_4\text{H}_3\text{S}\cdot\text{SO}_3\text{H}$   
 2-4(-pyridyl)-ethyl sulphonate  $\text{C}_5\text{H}_4\text{N}\cdot\text{CH}_2\text{CH}_2\text{SO}_3\text{H}$   
 In all cases the free sulphonics and their alkali metal, ammonium, magnesium and nickel salts are the full equivalents of each other in this invention.

5 Of the compounds in Table II we found the sodium salt of naphthalene 1:3:6-trisulphonate acid particularly effective when used at between 1-30 g./l.

10 If a group "B" material is used alone only a poor semi-bright deposit is obtained. When used in conjunction with the borated product, brilliant fully bright deposits are obtained. Good levelling is also obtained from using this product.

15 The concentration of the borated product is very wide, a certain minimum concentrated of the compounds of Table II being required depending on the concentration of group "A" compounds of Table I.

20 Brilliant nickel deposits may be obtained in accordance with this invention, using electrolytes listed in Table III.

TABLE III.—BATH CONCENTRATIONS IN GRAMS PER LITRE

| Bath                                                                   | 1         | 2    | 3      | 4      | 5      | 6      | 7    |
|------------------------------------------------------------------------|-----------|------|--------|--------|--------|--------|------|
| Nickel sulphate, $\text{NiSO}_4\cdot 7\text{H}_2\text{O}$              | 240-330   | 330  | 330    | 330    | 0-37.5 | 0-37.5 | 240  |
| Nickel chloride, $\text{NiCl}_2\cdot 6\text{H}_2\text{O}$              | 30-45     |      |        |        |        |        | 30   |
| Nickel formate, $\text{Ni}(\text{OOCCH}_3)_2\cdot 2\text{H}_2\text{O}$ |           |      |        |        |        |        | 45   |
| Nickel fluoroborate, $\text{Ni}(\text{BF}_4)_2$                        |           |      |        |        | 210    |        |      |
| Nickel sulphamate, $\text{Ni}(\text{O}_3\text{SNH}_2)_2$               |           |      |        |        | 225    |        |      |
| Sodium chloride, $\text{NaCl}$                                         |           |      | 29.5   |        |        |        |      |
| Sodium bromide, $\text{NaBr}$                                          |           |      |        |        |        |        |      |
| Boric acid, $\text{H}_3\text{BO}_3$                                    | 30-37.5   | 37.5 | 0-37.5 | 0-37.5 | 30     | 30     | 37.5 |
| 2-butyne 1:4 diol borate derivative                                    | (0.2-0.4) | 0.2  | 0.2    | 0.2    | 0.25   | 0.3    | 0.6  |
| 1,3,6 naphthalene trisulphonate sodium salt                            | 1-5       | 4.0  | 4.0    | 4.0    | 2.0    | 2.0    | 2.0  |
| Temperature, °C                                                        | 25-60     | 50   | 50     | 50     | 50     | 50     | 80   |

1:5 or 2:7 naphthalene disulphonate  $\text{C}_{10}\text{H}_6(\text{SO}_3\text{H})_2$

1:5 or 2:7 naphthalene disulphonate nickel salt  
 $\text{C}_{10}\text{H}_6(\text{SO}_3\text{H})_2\text{Ni}$

Naphthalene trisulphonate  $\text{C}_{10}\text{H}_5(\text{SO}_3\text{H})_3$

Naphthalene trisulphonate trisodium salt  
 $\text{C}_{10}\text{H}_5(\text{SO}_3\text{Na})_3$

Diphenyl pp-disulphonate  $\text{HSO}_3\text{C}_6\text{H}_4-\text{C}_6\text{H}_4\text{SO}_3\text{H}$

2-naphthol 3:6 disulphonate  $\text{HOC}_{10}\text{H}_5(\text{SO}_3\text{H})_2$

2-naphthol 3:6 disulphonate sodium salt

$\text{HOC}_{10}\text{H}_5(\text{SO}_3\text{Na})_2$

1-naphthylamino-3:6:8-trisulphonate

$\text{H}_2\text{N}\cdot\text{C}_{10}\text{H}_4(\text{SO}_3\text{H})_3$

(5) Heterocyclic sulphonics and alkali metal ammonium, magnesium and nickel salts thereof.

Sodium thiophene sulphonate  $\text{C}_4\text{H}_3\text{S}\cdot\text{SO}_3\text{Na}$

35 An example of the type of nickel solution that has been used with particular success in accordance with this invention is one containing:

|                                      |       |     |
|--------------------------------------|-------|-----|
| NiSO <sub>4</sub> ·7H <sub>2</sub> O | g./l. | 280 |
| NaCl                                 | g./l. | 40  |
| H <sub>3</sub> BO <sub>3</sub>       | g./l. | 40  |
| Naphthalene trisulphonate            | g./l. | 10  |

40 Sodium salt: 0.25 g./l. of the acetylenic borate reaction produce pH-3.6 and operated at 50° C. at 40-60 amperes per square foot.

45 Brilliant nickel deposits may be obtained in accordance with the invention from the electrolytes listed in Table 4 and Table 5.

TABLE 4.—BATH CONCENTRATIONS IN GRAMS PER LITRE

| Bath                                                                   | 1        | 2        | 3        | 4        | 5        | 6        | 7        |
|------------------------------------------------------------------------|----------|----------|----------|----------|----------|----------|----------|
| Nickel sulphate, $\text{NiSO}_4\cdot 7\text{H}_2\text{O}$              | 240-330  | 330      | 330      | 330      | 0-37.5   | 0-37.5   | 240      |
| Nickel chloride, $\text{NiCl}_2\cdot 6\text{H}_2\text{O}$              | 30-45    |          |          |          |          |          | 30       |
| Nickel formate, $\text{Ni}(\text{OOCCH}_3)_2\cdot 2\text{H}_2\text{O}$ |          |          |          |          |          |          | 45       |
| Nickel fluoroborate, $\text{Ni}(\text{BF}_4)_2$                        |          |          |          |          | 210      |          |          |
| Nickel sulphamate, $\text{Ni}(\text{O}_3\text{SNH}_2)_2$               |          |          |          |          | 225      |          |          |
| Sodium chloride, $\text{NaCl}$                                         |          | 15-30    |          |          |          |          |          |
| Sodium bromide, $\text{NaBr}$                                          |          |          | 51.5     |          |          |          |          |
| Boric acid, $\text{H}_3\text{BO}_3$ (saturation solution)              | 50-      | 50-      | 50-      | 50-      | 50-      | 50-      | 50-      |
| Reaction product of 2-butyne-1:4-diol and sodium perborate             | .005-0.3 | .005-0.3 | .005-0.3 | .005-0.3 | .005-0.3 | .005-0.3 | .005-0.3 |
| O-Sulphobenzoic acid imide sodium salt gm./litr.                       | 1-10     | 1-10     | 1-10     | 1-10     | 1-10     | 1-10     | 1-10     |
| Temperature, °C                                                        | 50-52    | 52       | 52       | 52       | 52       | 52       | 52       |
| 2-propene-1-sulphonic acid sodium salt                                 | 0.05-1.5 | 0.1-1.5  | 0.02-1.5 | 0.1-1.5  | 0.1-1.5  | 0.1-1.5  | 0.05-1.5 |

TABLE 5

| Bath                                                                   | 1        | 2        | 3        | 4        | 5        | 6        | 7        |
|------------------------------------------------------------------------|----------|----------|----------|----------|----------|----------|----------|
| Nickel sulphate, $\text{NiSO}_4\cdot 7\text{H}_2\text{O}$ gm./litr.    | 50/100   | 50/100   | 50/100   | 50/100   | 50/100   | 50/100   | 50/100   |
| Nickel chloride, $\text{NiCl}_2\cdot 6\text{H}_2\text{O}$ gm./litr.    | 150/300  | 150/300  | 150/300  | 150/300  | 150/300  | 150/300  | 150/300  |
| Nickel formate, $\text{Ni}(\text{OOCCH}_3)_2\cdot 2\text{H}_2\text{O}$ |          |          |          |          |          |          | 45       |
| Nickel fluoroborate, $\text{Ni}(\text{BF}_4)_2$                        |          |          |          |          | 210      |          |          |
| Nickel sulphamate, $\text{Ni}(\text{O}_3\text{SNH}_2)_2$               |          |          |          |          | 225      |          |          |
| Sodium chloride, $\text{NaCl}$                                         |          | 15-30    |          |          |          |          |          |
| Sodium bromide, $\text{NaBr}$                                          |          |          | 51.5     |          |          |          |          |
| Boric acid, $\text{H}_3\text{BO}_3$ saturation solution                | 50-      | 50-      | 50-      | 50-      | 50-      | 50-      | 50-      |
| Reaction product of 2-butyne-1:4-diol and sodium perborate             | .005-0.3 | .005-0.3 | .005-0.3 | .005-0.3 | .005-0.3 | .005-0.3 | .005-0.3 |
| O-Sulphobenzoic acid imide sodium salt gm./litr.                       | 1-10     | 1-10     | 1-10     | 1-10     | 1-10     | 1-10     | 1-10     |
| Temperature, °C                                                        | 50-52    | 50-52    | 50-52    | 50-52    | 50-52    | 50-52    | 50-52    |
| 2-propene-1-sulphonic acid sodium salt                                 | 0.05-1.5 | 0.1-1.5  | 0.02-1.5 | 0.1-1.5  | 0.1-1.5  | 0.1-1.5  | 0.05-1.5 |

According to one desirable process in accordance with this invention the solution comprises at least one nickel salt, in which is dissolved from 0.00156 to 0.3 g./l. of a reaction product of 2-butyne-1: 4-diol and sodium perborate and 0.1 to 1.0 g./l. 2-propene-1-sulphonic acid in the presence of between 50 g./l. and a saturated solution of boric acid and 0.5 to 80 g./l. of a water soluble sulphonyl oxygen compound selected from the group consisting of mononuclear and binuclear aromatic sulphonic acids, alkali metal, ammonium, magnesium and nickel salts of said acids and mononuclear aromatic sulphonamides and sulphonimides or salts of such amides and imides.

Examples of the type of nickel solutions that were used with particular success in accordance with this invention are those containing:

(1) 280 g./l.  $\text{NiSO}_4 \cdot 7\text{H}_2\text{O}$ : 40 g./l.  $\text{NaCl}$ : 56.25 g./l.  $\text{H}_3\text{BO}_3$ : 35 g./l. naphthalene trisulphonic acid-sodium salt. pH 3.6, temp. 48-56° C. Current density—40-100 amps/square foot. 0.3 g./l. of reaction product of 2-butyne-1: 4-diol and sodium perborate: 2-propene-1-sulphonic acid—1.0 g./l.

(2) 280 g./l.  $\text{NiSO}_4 \cdot 7\text{H}_2\text{O}$ : 40 g./l.  $\text{NaCl}$ : 56.25 g./l.  $\text{H}_3\text{BO}_3$ : 2 g./l. of o-sulphobenzoic acid imide sodium salt. pH 3.6. Temp. 48-56° C. Current density—40-100 amps/square foot. 0.3 g./l. of reaction product of 2-butyne-1: 4-diol and sodium perborate: 2-propene-1-sulphonic acid—1.0 g./l.

I claim:

1. A process for producing bright nickel deposits which comprises electro-depositing nickel from an aqueous acidic solution of at least one nickel salt in which there is dissolved from 0.00156 to 1.0 g./l. of a preformed borate compound consisting of the reaction product of the reaction of equal molar amounts of an acetylene alcohol and an alkali metal perborate at a temperature of 85-95° C.; together with a water-soluble sulphonyl oxygen compound at a concentration of from 0.5 to 90 g./l.

2. A process according to claim 1, wherein the acetylenic alcohol is 2-butyne-1:4-diol.

3. A process according to claim 2, wherein the amount of reacted 2-butyne-1:4-diol and sodium perborate is in the range of 0.01 to 0.5 g./l. and the amount of the sulphonyl oxygen compound is in the range of 0.5 to 80 g./l.

4. A process as claimed in claim 1 wherein the acetylenic alcohol is 3-pentyne-1-ol.

5. A process as claimed in claim 1 wherein the acetylenic alcohol is 2-methyl-3-butyne-2-ol.

6. A process as claimed in claim 1 wherein the acetylenic alcohol is 1-pentyne-3-ol.

7. A process as claimed in claim 1 wherein the acetylenic alcohol is 2-pentyne-1:4-diol.

8. A process according to claim 1 wherein the sulphonyl oxygen compound is selected from a group consisting of mononuclear and binuclear sulphonic acids, heterocyclic sulphonic acids, mononuclear aromatic sulphonic acids, alkali metal, ammonium, magnesium and nickel salts of said acids, and mononuclear aromatic sulphonamides and sulphonimides.

9. A process according to claim 1 wherein the sulphonyl oxygen compound is naphthalene trisulphonic acid sodium salt.

10. A process of producing bright nickel deposits which comprises electrodepositing nickel from an aqueous acidic solution of at least one nickel salt in which there is incorporated from 0.00156 to 0.3 g./l. of the borate reaction product of the reaction of equal molar amounts of an acetylenic alcohol and with sodium perborate at a temperature of 85-95° C., the said acetylenic alcohol having the general formula



15 where  $\text{M}_1$  is a hydroxyl, hydroxymethyl or hydroxyethyl radical,  $\text{M}_2$  is a hydrogen or methyl radical and  $\text{M}_3$  is a methyl, hydroxymethyl, hydroxyethyl, methoxymethyl, diethylaminomethyl, morpholinomethyl or hydroxypropyne radical and 0.5 to 90 g./l. of a water soluble sulphonyl oxygen compound.

11. A process for producing bright nickel deposits which comprises, electro-depositing nickel from an aqueous acidic solution of at least one nickel salt, in which is dissolved from 0.00156 to 0.3 g./l. of a borate reaction product of the reaction of equal molar amounts of 2-butyne-1:4-diol and sodium perborate at a temperature of 85-95° C. and 0.1 to 1.0 g./l. 2-propene-1-sulphonic acid in the presence of between 50 g./l. and a saturated solution of boric acid and 0.5 to 80 g./l. of a water soluble sulphonyl oxygen compound selected from the group consisting of mononuclear and binuclear aromatic sulphonic acids, alkali metals, ammonium, magnesium and nickel salts of said acids and mononuclear aromatic sulphonamides and imides or salts of such amides and imides.

12. A process for producing bright nickel deposits which comprises, electro-depositing nickel from an aqueous acidic nickel solution of at least one nickel salt in which there is dissolved from 0.00156 to 0.3 g./l. of the borate reaction product of the reaction of equal molar amounts of 2-butyne-1:4-diol and sodium perborate at a temperature of 85-95° C., 0.1 to 1.5 g./l. 2-propene-1-sulphonic acid, 50 g./l. to a saturated solution of boric acid and 0.5 to 80 g./l. of naphthalene trisulphonic acid-sodium salt.

13. A process for producing bright nickel deposits which comprises, electro-depositing nickel from an aqueous acidic solution of at least one nickel salt in which there is dissolved at least 0.3 g./l. of the borate reaction product of the reaction of equal molar amounts of 2-butyne-1:4-diol and sodium perborate at a temperature of 85-95° C., 0.1 to 1.0 g./l. 2-propene-1-sulphonic acid, at least 50 g./l. boric acid and 1 to 10 g./l. of ortho-sulphobenzoic acid imide sodium salt.

#### References Cited

#### UNITED STATES PATENTS

3,245,887 4/1966 Passal et al. 204—49

60 JOHN H. MACK, Primary Examiner  
G. L. KAPLAN, Assistant Examiner